# EUROPEAN PATENT SPECIFICATION

(11) **EP 0 662 169 B1**
(45) Date of publication and mention of the grant of the patent: **06.11.1996**
(21) Application number: 92918282.2
(22) Date of filing: 11.08.1992
(51) Int. Cl.: D21C 3/24

(54) **A PROCESS FOR THE CONTINUOUS DIGESTION OF CELLULOSIC FIBER MATERIAL**
VERFAHREN ZUM KONTINUIERLICHEN AUFSCHLIESSEN VON ZELLULOSEFASERN
PROCEDE DE LESSIVAGE CONTINU DE MATERIAU EN FIBRE CELLULOSIQUE

(30) Priority: 23.08.1991 SE 9102427
(43) Date of publication of application: 12.07.1995
(73) Proprietor: KAMYR Aktiebolag, 651 15 Karlstad (SE)
(72) Inventor: BACKLUND, Ake, S-652 24 Karlstad (SE)
(74) Representative: Lundquist, Lars-Olof
(86) International application number: SE9200546
(87) International publication number: WO9304232

(56) References cited:
- DE-A- 3 938 504
- US-A- 3 802 956

## Description

The present invention relates to a process for the continuous digestion of cellulosic fiber material, comprising impregnation with impregnating liquid consisting of at least one fresh digesting liquor, in a closed impregnating system and subsequent digestion with digesting liquid in a closed digester system, said impregnating liquid being added through a supply system, together with steamed fibre material, to an inlet end of the impregnating system, liquid being withdrawn from the impregnating system at a point located at a predetermined distance from said inlet end.

When feeding wood chips, for instance, into a continuous digester a certain minimum quantity of liquid must be added through the supply system together with the chips. If too little liquid is added in relation to the quantity of chips the temperature will become too high in the supply system and the sinking rate of the chips in the impregnating vessel or digester will be disturbed. The requisite amount of liquid is normally obtained with the digesting liquor, e.g. white liquor, added to the supply system for impregnating the chips. If necessary spent digesting liquid (black liquor), the temperature of which has been lowered through relief in several steps or by means of indirect cooling, may be returned to the supply system, thus increasing the amount of liquid available. In certain multi-step processes in which the first step is impregnation or digestion with a different chemical from that used in subsequent digestion step or where for technical reasons it is unsuitable to use fully spent digesting liquid (black liquor), the requirement for a certain minimum quantity of liquid must be fulfilled by adding a sufficient amount of the digesting liquid from the first step, possibly diluted with water. This entails several drawbacks such as poorer heat economy due to the increased consumption of steam in subsequent cooking steps and/or increased need for evaporation for recovery of the chemicals. Another drawback may be that the concentration of the cooking chemicals in first step becomes too low to achieve the desired effect of the process. Addition of black liquor to the supply system is described in US-A-3802956 and DE-A-3938504. In the processes according to said documents liquid is withdrawn from the impregnation system at a point located at a predetermined distance from the inlet end, and the liquid withdrawn is mixed with black liquor.

The liquid to wood ratio at the inlet to a continuous digester is normally 3.0 - 3.5 m³ per ton dry chips. In conventional sulphate cooking 70-100% of the white liquor required is normally added to the supply system for the impregnating vessel via a high-pressure pump. The amount of liquid at the inlet to the impregnating vessel may then be within an interval of about 2.4 - 2.8 m³ per ton dry chips, distributed as follows:

| | | |
|---|---|---|
| A | Chips moisture (moisture content 50 %) | 1.0 m³ |
| B+C | Steam condensate | 0.3 m³ |
| E | White liquor (70-100%) | 1.1-1.5 m³ |

As mentioned above, black liquor can be added to the impregnating vessel through the supply system in order to increase the liquid to wood ratio, for instance to 3.0 m³ or above. The temperature of the black liquor should not exceed 100 C°. If too little liquid is added to the impregnating vessel, disturbances will result in the supply system due to the formation of steam in the down pipe located before the high pressure valve. The temperature of the liquid exceeds the temperature corresponding to the steam pressure in the pressure steaming vessel located upstream. Sinking of the chips in the impregnating vessel is also impeded. The quantity of free liquid, i.e. the portion of liquid which is not absorbed by the chips, becomes too low and the flow rate of the liquid is correspondingly reduced. The flow rate of the free liquid exerts a driving force on the column of chips. It is important that this driving force is great in the upper part of the impregnating vessel where the chips are still not saturated with liquid but have a tendency to float. This requirement is of less importance in the lower part of the impregnating vessel since by this stage the chips are substantially saturated with liquid and therefore tend to sink due to their own weight. When treatment is carried out in several steps using different digesting liquids in the various steps, there is the same need to maintain a sufficiently high liquid to wood ratio in the first step, i.e. in the initial concurrent flow zone in the impregnating vessel. However, it may be that the process or operating economy requires that the digesting liquid of the first step has to be added in a limited quantity, in which case it may be difficult to achieve a sufficiently high liquid to wood ratio. At the same time, the liquid flow at the entrance to the digester must be controlled so that it does not become too great since this results in too great a consumtion of high-pressure steam in heat exchanger present in the transfer system and of direct steam to the top of the digester. Furthermore, the withdrawal strainer in the upper part of the countercurrent flow washing zone of the digester becomes overloaded.

The object of the present invention is to eliminate said problems and provide a simple and reliable method of maintaining a sufficiently high flow of liquid in at least the initial part of the impregnating vessel without the liquid flow in the digester becoming too high. In other words, the invention aims to solve the problems existing when black liquor cannot be used in order to provide a sufficiently high liquid to wood ratio in the impregnating vessel without such ratio being too high in the digester.

The process according to the invention is characterised in that such a first quantity of liquid (F) is whithdrawn at said withdrawal point and recirculated directly to the supply system that a predetermined minimum ratio between liquid and fibre material is continuously maintained in the impregnating system prior to said withdrawal point, the liquid in said liquid to fibre material ratio being derived from original moisture (A) in the fibre material, condensates (B, C) from an initial steaming of the fibre material, and added fresh digesting liquor(s) (D and/or E) besides said withdrawn and recirculated quantity of liquid (F). The term "directly" as used herein means that the liquid is recirculated as such to the supply system, i.e. without being mixed with black liquor.

The invention will be described in more detail in the following with reference to the drawing which shows schematically a flow diagram of a plant for the continuous digesting of cellulosic fiber material in the form of wood material which has been disintegrated to chips.

The plant shown in the drawing comprises a vertical steaming vessel 1, a horizontal steaming vessel 2, a vertical impregnating vessel 3 and a vertical digester 4. Chips are fed through a pipe 5 to the vertical steaming vessel 1, to which low pressure steam is supplied through a pipe 6 in order to heat the chips and reduce their air content. This pre-steaming process is performed at atmospheric pressure. The heated chips are dosed by a chip meter disposed in a connection 7 between the two steaming vessels, said connection 7 also containing a lower-pressure valve 8 which locks through the chips into the horizontal steaming vessel 2. Low-pressure steam is added through a pipe 9. The pressure in this second steam vessel 2 is 1-1.5 bar over-pressure. From the pressure steaming vessel 2, the chips fall into a down pipe 10 with a high pressure valve 11 disposed at the lower end thereof. A liquid level is maintained in the down pipe 10. The high pressure valve 11 is provided with a rotor having pockets. One pocket is always in low pressure position to be in open communication with the pre-steaming vessel 1, and another pocket is always simultaneously in high pressure position to be in open communication with the impregnating vessel 3 via a supply pipe 12 connected to the top of the impregnating vessel 3. Liquid in a circulation loop 13 provided with a pump 20 feeds the chips from the down pipe 10 into the high pressure valve 11 and fills one of the rotor pockets. A screen is mounted in the housing of the high pressure valve 11 to prevent chips from accompanying the circulation liquid in the circulation loop 13. The liquid displaced by the chips in the high pressure valve 11 is withdrawn from the circulation loop 13 by means of a screen 14 disposed therein, from which the liquid withdrawn is conducted to a level tank 15 via a pipe 16. The level tank 15 is connected to the top of the impregnating vessel 3 by a pipe 17 containing a high-pressure pump 18 to pump the liquid withdrawn into the impregnating vessel 3.

The high pressure valve 11 and impregnating vessel 3 are connected by means of a circulation loop comprising said supply pipe 12 which is connected to the top of the impregnating vessel 3, and a return pipe 21 which connects the top of the impregnating vessel to the high pressure valve 11 to return liquid separated off by a top separator disposed in the impregnating vessel 3. The liquid is caused to circulate by means of a pump 22 located in the return pipe 21. When a filled rotor pocket arrives in the high pressure position, i.e. in direct communication with the circulation loop 12, 21, it is rinsed clean by the return liquid in this circulation loop. The flow rate of the return liquid is so high that it flushes the chips from the rotor pocket with it into the impregnating vessel 3. The pressure in the impregnating vessel 3 is normally 8-15 bar over-pressure. However, for certain processes it may be as high as 15-45 bar over-pressure.

Fresh digesting liquor D from a first storage tank is fed to the top of the impregnating vessel 3 via a pipe 23. The pipe 23 is suitably connected to the pipe 17 from the level tank 15 so that the high-pressure pump 18 is utilized for pumping both the liquid withdrawn from the first circulation loop 13, and the digesting liquor D which thus constitutes fresh impregnating liquid.

Fresh digesting liquor E is fed to the digester from a second storage tank via a pipe 24 containing a high-pressure pump 25. Some of the digesting liquor E may be used as impregnating liquid and be fed to the top of the impregnating vessel 3 via a branch pipe 26 provided with a valve. This branch pipe 26 is suitably connected to the pipe 17 from the level tank 15. The impregnated chips are transferred from the bottom of the impregnating vessel 3 to the top of the digester 4 via a pipe 27. A strainer is mounted at the top of the digester 4 to separate off a certain amount of liquid which is then returned to the bottom of the impregnating vessel 3 via a return pipe 28 containing a pump 29 to pump the chips to the digester 4 with the aid of the separated liquid. The return pipe 28 passes a heat exchanger 30 to heat the liquid passing it by the supply of high-pressure steam via a pipe 31. The supply pipe 27 and return pipe 28 form a transfer circulation for the suspension of impregnated chips and boiling liquid. A larger quantity of digesting liquor E is added to said transfer circulation in that the pipe 24 for the digesting liquor is connected to the return pipe 28 before pump 29. If desired, a smaller quantity of the digesting liquor may be added to a circulation pipe 33 of the digester, via a pipe 19 provided with a valve. The digester is provided with a strainer 32 for circulation of liquid through pipe 33 with the aid of a pump 34, the liquid being heated in a heat exchanger 35. The pipe 33 comprises a central tube disposed in the centre of the digester with its orifice at the strainer 32. The digested chips are washed in countercurrent flow in the lower part of the digester, using washing liquid supplied through a pipe 36 and pumped by a high-pressure pump 37 into the lower part of the digester in an amount which is regulated to ensure that the digester is kept filled with liquid. The washing liquid is heated indirectly by steam which is supplied to a heat exchanger 38 disposed in a pipe 39 for circulation of washing liquid by means of a pump 40. The washing liquid is removed through a strainer 41 and returned through a central pipe extending from the bottom of the digester and having its orifice at a strainer 41. The washing liquid heated in this manner is forced to flow in countercurrent up through the chips column as it moves slowly downwards, thereby displacing its content of spent digesting liquor which is withdrawn through a strainer 42 and conducted via a pipe 43 to a flash cyclone (not shown) and a recovery plant (not shown). The digested chips are fed out at the bottom of the digester using suitable scrapers, and is conducted through a pipe 44 for continued processing. Besides indirect heating of digesting liquid and wood in said transfer circulation 27, 28, indirect heating is also performed with steam supplied to the top of the digester through a pipe 45.

According to the present invention the impregnating vessel is provided with a strainer 46 disposed at a predetermined distance from the top of the impregnating vessel as seen from the point where the chips are supplied, i.e. the inlet end. According to the present invention, furthermore, a return pipe 47 provided with a valve is connected between this strainer 46 and the top of the impregnating vessel in order to return a predetermined quantity of liquid to the start of the impregnating zone. The return pipe 47 contains a high-pressure pump 48 and passes through a heat exchanger 49, the other fluid side of which is connected to the pipe 24 for fresh digesting liquor E via branch pipes 50, 51. The flow to the heat exchanger 49 is regulated by a valve 52 in the pipe 24 for fresh digesting liquor E. The return pipe 47 is connected to the pipe 17 from the level tank 15 at a point located before the high-pressure pump 18.

The following example further illustrates the invention.

The impregnating liquid D is added in an amount of about 0.7 m³ per ton dry wood. The quantity of liquid A from chips moisture is about 1.0 m³ and from the steam condensates B and C about 0.3 m³ per ton dry wood. These three sources of liquid thus supply about 2.0 m³ per ton dry wood to the top of the impregnating vessel 3. Liquid F is withdrawn from the strainer 46 in the impregnating vessel in an amount of about 1.0 m³ per ton dry wood. The liquid F withdrawn is cooled to a suitable temperature in the cooler 49 in order to avoid disturbances in the supply system. The total amount of the liquids A, B, C, D and F is thus about 3.0 m³ per ton dry wood. This quantity of liquid is sufficient to provide a constant downward movement of the chips column in the impregnating vessel 3. The amount of liquid F may be varied within wide limits, depending on the other liquid flows to the impregnating vessel and on other operating conditions. Digesting liquor E in the form of white liquor is supplied to the digester 4 via pipes 24, 28, 27 and 19 in an amount of about 1.5 m³ per ton dry chips. All together about 3.5 m³ liquid per ton dry chips is thus transferred to the digester, i.e. the sum of the liquid quantities A, B, C, D and E. This gives an acceptable flow of liquid in the digester 4 with respect to heat economy and operating reliability.

When the process is repeated without withdrawing and returning liquid F (the valve in pipe 47 is closed), the amount of fresh digesting liquor D must be increased from 0.7 to 1.7 m³ per ton dry chips, thus giving a total flow of liquid to the digester of 4.5 m³ per ton dry chips. However, such a run is unsuitable in practice since the large flow of liquid causes too high a consumption of high-pressure steam in the heat exchanger 30 in the transfer system and of direct steam to the top of the digester. The strainer in the upper part of the countercurrent flow washing zone of the digester also becomes overloaded.

The temperature at the top of the impregnating vessel is generally about 110-120 C° and at the bottom, i.e. in the transfer circulation 27, 28, about 130-160 C°. The liquid withdrawn through the strainer 46 has a temperature of about 120-130 C°, while the black liquor withdrawn from the digester through the strainer 42 has a temperature of about 150-170 C°.

The method according to the invention for maintaining a sufficiently high flow of liquid in the upper part of the impregnating vessel can be utilized for various embodiments of the digesting process. The fresh digesting liquor D, for instance, may consist of an alkaline solution with a high sodium sulphide content or of only sodium sulphide. Sodium sulphide is consumed to a relatively small extent during impregnation conditions and a sufficiently high sodium sulphide content can therefore be maintained even if impregnating liquid F is withdrawn and returned to the inlet of the impregnating vessel. The fresh digesting liquor E may consist of ordinary white liquor, i.e. a mixture of substantially sodium sulphide and sodium hydroxide, or a white liquor containing substantially sodium hydroxide.

In the case the chips are impregnated with a part of the fresh digesting liquor E and no other fresh digesting liquor D is added, a sufficient flow of liquid will be obtained at the beginning of the impregnating vessel by withdrawing a sufficient quantity of liquid F from the impregnating vessel 3 and returning it via the supply system. The fresh digesting liquor E required for the rest of the process is added to the digester 4 via the transfer circulation 27, 28 and/or the circulation 33 described or some other circulation of digesting liquid in the digester vessel.

The liquid F withdrawn from the initial concurrent flow impregnating zone may be large enough to correspond to all the free liquid. The liquid bound by the chips is about 1.8 m³ per ton dry wood in the case of softwood and about 1.0-1.5 m³ per ton dry wood in the case of hardwood, depending on the density of the chips. Withdrawing additional liquid through strainer 46 will cause liquid to flow upwardly from the bottom of the impregnating vessel towards the strainer 46. In such an operation some of the digesting liqour E which has been added to the transfer circulation will meet the chips in countercurrent flow, thereby resulting in improved impregnation. The additional liquid withdrawn from the lower countercurrent flow impregnating zone via the strainer 46 can be returned to the transfer circulation 27, 28 or be used in som other way. It is thus not included when calculating the amount of liquid F which is withdrawn and returned to the supply system.

Circulating a considerable proportion of the impregnating liquid back to the supply system increases the concentration of the fresh digesting liquor D when this is used, thus producing improved impregnating results, particularly when the fresh digesting liquor D consists of a polysulphide solution or a solution containing anthraquinone. As mentioned earlier, the temperature in the impregnating vessel 3 can advantageously be regulated to a suitable level by cooling the withdrawn impregnating liquid F in the cooler 49.

The fresh digesting liquor D may also consist of an organic substance, such as methanol or ethanol, to impregnate the steamed chips, possibly in the presence of a small quantity of fresh digesting liquor E, e.g. white liquor. The rest of the fresh digesting liquor E is then added to the transfer circulation 27, 28 and/or one of the liquid circulations, e.g. 33, of the digester.

The process according to the invention is also applicable to sulphite digestion in several steps, for instance acid sulphite digestion. Neither is it limited to a continuous digester with separate impregnating vessel, but may be used in a digester vessel for the continuous digesting with initial impregnating zone, such as a one-vessel hydraulic digester.

The impregnating liquid F withdrawn may alternatively be returned to the supply system at a point in the pipe 17 located after the high-pressure pump 18. This reduces the need of pump energy.

If the liquid F withdrawn is enriched with gas, which may cause operating disturbance, it may be suitable to flash the liquid to a low pressure for degassing before feeding it to the sypply system.

As will be understood from the above description and following claims no black liquor is added to the supply system of the impregnating system.

## Claims

1. A process for the continuous digestion of cellulosic fiber material, comprising impregnation with impregnating liquid consisting of at least one fresh digesting liquor, in a closed impregnating system and subsequent digestion with digesting liquid in a closed digester system, said impregnating liquid being supplied through a supply system, together with steamed fibre material, to an inlet end of the impregnating system, liquid being withdrawn from the impregnating system at a point (46) located at a predetermined distance from said inlet end, characterized in that such a first quantity of liquid (F) is withdrawn at said withdrawal point (46) and recirculated directly to the supply system that a predetermined minimum ratio between liquid and fibre material is continuously maintained in the impregnating system prior to said withdrawal point(46), the liquid in said liquid to fibre material ratio being derived from original moisture (A) in the fibre material, condensates (B, C) from an initial steaming of the fibre material, and added fresh digesting liquor(s) (D and/or E) besides said withdrawn and recirculated quantity of liquid (F).

2. A process as claimed in claim 1, characterized in that said liquid to fibre material ratio is at least 2.5:1, preferably at least 3.0:1, calculated on dry fibre material.

3. A process as claimed in claim 1 or 2, characterized in that the fresh digesting liquor (E) added through the supply system consists chemically of the same fresh digesting liquor (E) supplied to the digester system.

4. A process as claimed in claim 1 or claim 2, characterized in that a fresh digesting liquor (D) having a different chemical composition from the fresh digesting liquor (E) added to the digester system, is added to the supply system.

5. A process as claimed in claim 4, characterized in that a part of the fresh digesting liquor (E) for the digester system is also added to the supply system.

6. A process as claimed in any of claims 1-5, characterized in that the temperature in the impregnating system is regulated by causing the first quantity of liquid (F), which is withdrawn and recirculated, to pass a heat exchanger (49) before being introduced into the supply system.

7. A process as claimed in claim 6, characterized in that the digesting liquid which is added to the digester system or water for the production of hot water is used as heat-exchange medium.

8. A process as claimed in claim 4 or 5, characterized in that a neutral or alkaline solution of sodium sulphide, a solution of an organic compound such as methanol and ethanol, a solution of polysulphide or a solution of anthraquinone is used as said digesting liquor (D) of different chemical composition.

9. A process as claimed in any of claims 1-8, characterized in that the quantity of liquid (F) withdrawn and recirculated to the supply system is equivalent to the quantity of free liquid in the impregnating system before the withdrawal point (46).

10. A process as claimed in claim 9, characterized in that a countercurrent flow is maintained downstream of the withdrawal point (46), seen in relation to the movement of the fibre material, by withdrawing a second quantity of liquid from the impregnating system over and above said free liquid (F), said second quantity of liquid constituting a part of a liquid which is introduced at the outlet end of the impregnating system to transfer impregnated fibre material to the digester system.

## Patentansprüche

1. Verfahren zum kontinuierlichen Aufschluß von Zellulosefasermaterial, beinhaltend ein Tränken mit aus mindestens einer frischen Aufschließlauge bestehender Tränkflüssigkeit in einer geschlossenen Tränkanlage und einen nachfolgenden Aufschluß mit Aufschließflüssigkeit in einer geschlossenen Kocheranlage, wobei die Tränkflüssigkeit durch ein Zufuhrsystem zusammen mit gedämpftem Fasermaterial einem Einlaßende der Tränkanlage zugeführt wird, Flüssigkeit der Tränkanlage bei einem in vorgegebenem Abstand vom Einlaßende angeordneten Punkt (46) entnommen wird, dadurch gekennzeichnet, daß eine solche erste Menge Flüssigkeit (F) am Entnahmepunkt (46) entnommen und direkt zum Zufuhrsystem zurückgeleitet wird, daß in der Tränkanlage vor dem Entnahmepunkt (46) kontinuierlich ein vorgegebenes Mindestverhältnis zwischen Flüssigkeit und Fasermaterial aufrechterhalten wird, wobei die Flüssigkeit in dem Verhältnis Flüssigkeit zu Fasermaterial sich aus ursprünglicher Feuchtigkeit (A) im Fasermaterial, Kondensaten (B, C) aus einer ersten Dämpfung des Fasermaterials sowie zugegebener frischer Aufschließlauge bzw. zugegebenen frischen Aufschließlaugen (D und/oder E) neben der entnommenen und zurückgeführten Menge an Flüssigkeit (F) herleitet.

2. Verfahren nach Anspruch 1, dadurch gekennzeichnet, daß das Verhältnis Flüssigkeit zu Fasermaterial mindestens 2,5:1, vorzugsweise mindestens 3,0:1, bezogen auf trockenes Fasermaterial, beträgt.

3. Verfahren nach Anspruch 1 oder 2, dadurch gekennzeichnet, daß die durch das Zufuhrsystem hinzugefügte frische Aufschließlauge (E) chemisch aus der gleichen, der Kocheranlage zugeführten frischen Aufschließlauge (E) besteht.

4. Verfahren nach Anspruch 1 oder 2, dadurch gekennzeichnet, daß dem Zufuhrsystem eine frische Aufschließlauge (D) mit einer sich von der der Kocheranlage hinzugefügten frischen Aufschließlauge (E) unterscheidenden chemischen Zusammensetzung hinzugefügt wird.

5. Verfahren nach Anspruch 4, dadurch gekennzeichnet, daß ein Teil der frischen Aufschließlauge (E) für die Kocheranlage gleichfalls dem Zufuhrsystem hinzugefügt wird.

6. Verfahren nach einem der Ansprüche 1-5, dadurch gekennzeichnet, daß die Temperatur in der Tränkanlage geregelt wird, indem man die erste entnommene und zurückgeführte Menge Flüssigkeit (F) vor ihrer Einleitung in das Zufuhrsystem einen Wärmeaustauscher (49) passieren läßt.

7. Verfahren nach Anspruch 6, dadurch gekennzeichnet, daß die der Kocheranlage hinzugefügte Aufschließflüssigkeit oder Wasser zur Erzeugung von Heißwasser als Wärmeaustauschmedium eingesetzt wird.

8. Verfahren nach Anspruch 4 oder 5, dadurch gekennzeichnet, daß als die Aufschließlauge (D) einer unterschiedlichen chemischen Zusammensetzung eine neutrale oder alkalische Lösung von Natriumsulfid, eine Lösung einer organischen Verbindung wie Methanol und Ethanol, eine Lösung von Polysulfid oder eine Lösung von Anthrachinon eingesetzt wird.

9. Verfahren nach einem der Ansprüche 1-8, dadurch gekennzeichnet, daß die entnommene und zum Zufuhrsystem zurückgeführte Menge Flüssigkeit (F) der Menge an freier Flüssigkeit in der Tränkanlage vor dem Entnahmepunkt (46) äquivalent ist.

10. Verfahren nach Anspruch 9, dadurch gekennzeichnet, daß unterhalb des Entnahmepunkts (46), bezogen auf die Bewegung des Fasermaterials, eine Gegenströmung aufrechterhalten wird, indem der Tränkanlage über die freie Flüssigkeit (F) hinaus eine zweite Menge Flüssigkeit entnommen wird, die einen Teil einer Flüssigkeit ausmacht, die am Auslaßende der Tränkanlage eingeleitet wird, um getränktes Fasermaterial zur Kocheranlage zu transportieren.

## Revendications

1. Procédé de lessivage continu de matériau en fibre cellulosique, comprenant l'imprégnation à l'aide d'un liquide imprégnant se composant d'au moins une liqueur de lessivage fraîche, dans un système d'imprégnation clos, et un lessivage subséquent à l'aide d'un liquide de lessivage dans un système lessiveur clos, ledit liquide d'imprégnation étant alimenté à travers un système d'alimentation, conjointement à un matériau en fibre traité à la vapeur, à une extrémité d'entrée du système d'imprégnation, le liquide étant retiré du système d'imprégnation à un point (46) situé à une distance prédéterminée de ladite extrémité d'entrée, caractérisé en ce que l'on retire audit point de retrait (46) et en ce que l'on recycle directement dans le système d'alimentation une première quantité de liquide (F) telle qu'un rapport prédéterminé minimum entre liquide et matériau en fibre est maintenu en continu dans le système d'imprégnation avant ledit point de retrait (46), le liquide dans ledit rapport du liquide au matériau en fibre étant dérivé de l'humidité initiale (A) dans le matériau en fibre, des condensats (B, C) obtenus à partir d'un traitement à la vapeur initial du matériau en fibre, et de ou des liqueur(s) de lessivage fraîche(s) ajoutée(s) (D et/ou E) en plus de ladite quantité retirée et recyclée de liquide (F).

2. Procédé selon la revendication 1, caractérisé en ce que ledit rapport du liquide au matériau en fibre est au moins de 2,5:1, de préférence au moins de 3,0:1, calculé sur la base du matériau en fibre sec.

3. Procédé selon la revendication 1 ou 2, caractérisé en ce que la liqueur de lessivage fraîche (E), ajoutée à travers le système d'alimentation, se compose chimiquement de la même liqueur de lessivage fraîche (E), alimentée au système lessiveur.

4. Procédé selon la revendication 1 ou la revendication 2, caractérisé en ce qu'une liqueur de lessivage fraîche (D) ayant une composition chimique différente de celle de la liqueur de lessivage fraîche (E) ajoutée au système lessiveur, est ajoutée au système d'alimentation.

5. Procédé selon la revendication 4, caractérisé en ce qu'une partie de la liqueur de lessivage fraîche (E) pour le système lessiveur est également ajoutée au système d'alimentation.

6. Procédé selon l'une quelconque des revendications 1-5, caractérisé en ce que la température dans le système d'imprégnation est régulée en forçant la première quantité de liquide (F), qui est retirée et recyclée à passer dans une échangeur de chaleur (49) avant d'être introduite dans le système d'alimentation.

7. Procédé selon la revendication 6, caractérisé en ce que le liquide de lessivage qui est ajouté au système lessiveur ou à l'eau pour la production d'eau chaude, est utilisé en tant que milieu d'échange thermique.

8. Procédé selon la revendication 4 ou 5, caractérisé en ce qu'une solution neutre ou alcaline de sulfure de sodium, une solution d'un composé organique tel que le méthanol et l'éthanol, une solution de polysulfure ou une solution d'anthraquinone est utilisée en tant que ladite liqueur de lessivage (D) de composition chimique différente.

9. Procédé selon l'une quelconque des revendications 1-8, caractérisé en ce que la quantité de liquide (F), retirée et recyclée dans le système d'alimentation, est équivalente à la quantité de liquide libre dans le système d'imprégnation avant le point de retrait (46).

10. Procédé selon la revendication 9, caractérisé en ce qu'un écoulement à contre-courant est maintenu en aval du point de retrait (46), vu du point de vue du mouvement du matériau en fibre, en retirant une deuxième quantité de liquide du système d'imprégnation, en sus dudit liquide libre (F), ladite deuxième quantité de liquide constituant une partie d'un liquide qui est introduit à l'extrémité de sortie du système d'imprégnation pour transférer le matériau en fibre imprégné au système lessiveur.
